



US008105670B2

(12) **United States Patent**  
**Wu et al.**

(10) **Patent No.:** **US 8,105,670 B2**  
(45) **Date of Patent:** **\*Jan. 31, 2012**

(54) **GLYCOLURIL RESIN AND POLYOL RESIN DUAL MEMBERS**

(75) Inventors: **Jin Wu**, Webster, NY (US); **Jonathan H Herko**, Walworth, NY (US); **Scott J Griffin**, Fairport, NY (US); **Michael S Roetker**, Webster, NY (US); **Dennis J Prosser**, Walworth, NY (US); **Dante M Pietrantoni**, Rochester, NY (US)

(73) Assignee: **Xerox Corporation**, Norwalk, CT (US)

(\*) Notice: Subject to any disclaimer, the term of this patent is extended or adjusted under 35 U.S.C. 154(b) by 464 days.

This patent is subject to a terminal disclaimer.

(21) Appl. No.: **12/413,795**

(22) Filed: **Mar. 30, 2009**

(65) **Prior Publication Data**

US 2010/0248108 A1 Sep. 30, 2010

(51) **Int. Cl.**

**B32B 1/08** (2006.01)  
**B32B 27/08** (2006.01)  
**B32B 27/18** (2006.01)  
**B32B 27/28** (2006.01)

(52) **U.S. Cl.** ..... **428/35.7**; 428/411.1; 428/412; 428/421; 428/422; 428/473.5; 428/474.4; 428/522; 399/308

(58) **Field of Classification Search** ..... None  
See application file for complete search history.

(56) **References Cited**

U.S. PATENT DOCUMENTS

5,487,707 A 1/1996 Sharf et al.  
6,318,223 B1 11/2001 Yu et al.  
6,440,515 B1 8/2002 Thornton et al.  
6,602,156 B2 8/2003 Schlueter, Jr.  
7,031,647 B2 4/2006 Mishra et al.

7,130,569 B2 10/2006 Goodman et al.  
7,139,519 B2 11/2006 Darcy, III et al.  
7,910,183 B2 3/2011 Wu  
7,923,188 B2 \* 4/2011 Lin et al. ..... 430/59.6  
2004/0221942 A1 \* 11/2004 Yu et al. ..... 156/157  
2006/0002746 A1 1/2006 Darcy et al.  
2007/0248813 A1 \* 10/2007 Wu et al. ..... 428/337  
2008/0032218 A1 2/2008 Wu et al.  
2009/0035675 A1 2/2009 Wu  
2010/0247918 A1 9/2010 Wu  
2010/0247919 A1 9/2010 Wu  
2010/0248102 A1 9/2010 Wu  
2010/0248103 A1 9/2010 Wu  
2010/0248104 A1 9/2010 Wu  
2010/0248106 A1 9/2010 Wu  
2010/0248107 A1 9/2010 Wu et al.  
2010/0249322 A1 9/2010 Wu

FOREIGN PATENT DOCUMENTS

EP 1 612 617 A2 1/2006

OTHER PUBLICATIONS

Jul. 6, 2010 European Search Report issued in EP 10 15 6587.  
See the "Cross Reference to Related Applications" Section on pp. 1 and 2 of the Specification Being Filed Concurrently.

Jin Wu et al., U.S. Appl. No. 12/200,147 entitled Coated Seamed Transfer Member, filed Aug. 28, 2008.

Jin Wu et al., U.S. Appl. No. 12/200,179 entitled Coated Transfer Member, filed Aug. 28, 2008.

Jonathan Herko et al., U.S. Appl. No. 11/895,255 entitled Flexible Imaging Member Belt Seam Smoothing Process, filed Aug. 22, 2007.

Jin Wu, U.S. Appl. No. 12/129,995 on Polyimide Intermediate Transfer Components, filed May 30, 2008.

Jin Wu, U.S. Appl. No. 12/181,354, on Core Shell Intermediate Transfer Components, filed Jul. 29, 2008.

Jin Wu, U.S. Appl. No. 12/181,409 on Treated Carbon Black Intermediate Transfer Components, filed Jul. 29, 2008.

\* cited by examiner

*Primary Examiner* — Ramsey Zacharia

(74) *Attorney, Agent, or Firm* — Oliff & Berridge, PLC

(57) **ABSTRACT**

An intermediate transfer member, such as a belt, where the surface of the belt contains as a coating a mixture of a glycoluril resin and a polyol resin.

**21 Claims, No Drawings**

**GLYCOLURIL RESIN AND POLYOL RESIN  
DUAL MEMBERS**

**CROSS REFERENCE TO RELATED  
APPLICATIONS**

U.S. application Ser. No. 12/413,627, U.S. Publication No. 20100248103, filed Mar. 30, 2009, entitled Resin Mixture Backing Layer Containing Photoconductor, the disclosure of which is totally incorporated herein by reference, illustrates a photoconductor comprising a substrate, an imaging layer thereon, and a backing layer located on a side of the substrate opposite the imaging layer wherein the outermost layer of the backing layer adjacent to the substrate is comprised of a glycoluril resin, and a polyol resin mixture.

U.S. application Ser. No. 12/413,633, U.S. Publication No. 20100249322, filed Mar. 30, 2009, entitled Fluorinated Sulfonic Acid Polymer Grafted Polyaniline Containing Intermediate Transfer Members, the disclosure of which is totally incorporated herein by reference, illustrates an intermediate transfer member comprised of a substrate, and in contact therewith a polyaniline having grafted thereto a fluorinated sulfonic acid polymer.

U.S. application Ser. No. 12/413,638, U.S. Publication No. 20100247918, filed Mar. 30, 2009, entitled Perfluoropolyether.

Polymer Grafted Polyaniline Containing Intermediate Transfer Members, the disclosure of which is totally incorporated herein by reference, illustrates an intermediate transfer member comprised of a substrate and in contact with the substrate a polyaniline grafted perfluoropolyether phosphoric acid polymer.

U.S. application Ser. No. 12/413,642, U.S. Publication No. 20100247919, filed Mar. 30, 2009, entitled Fluorotelomer Grafted Polyaniline Containing Intermediate Transfer Members, the disclosure of which is totally incorporated herein by reference, illustrates An intermediate transfer member comprised of a substrate, and a layer comprised of polyaniline having grafted thereto a fluorotelomer.

U.S. application Ser. No. 12/413,645, now U.S. Patent 7,910,183, filed Mar. 30, 2009, entitled Layered Intermediate Transfer Members, the disclosure of which is totally incorporated herein by reference, illustrates an intermediate transfer member comprised of a polyimide substrate, and thereover a polyetherimide/polysiloxane.

U.S. application Ser. No. 12/413,651, U.S. Publication No. 20100248106, filed Mar. 30, 2009 entitled Polyimide Polysiloxane Intermediate Transfer Members, the disclosure of which is totally incorporated herein by reference, illustrates an intermediate transfer member comprised of at least one of a polyimide/polyetherimide/polysiloxane, and a polyimide polysiloxane.

U.S. application Ser. No. 12/413,783, U.S. Publication No. 20100248107, filed Mar. 30, 2009 entitled Glycoluril Resin And Polyol Resin Members, the disclosure of which is totally incorporated herein by reference, illustrates a process which comprises providing a flexible belt having at least one welded seam extending from one parallel edge to the other parallel edge, the welded seam having a rough seam region comprising an overlap of two opposite edges; contacting the rough seam region with a heat and pressure applying tool; and smoothing out the rough seam region with heat and pressure applied by the heat and pressure applying tool to produce a flexible belt having a smooth welded seam, and subsequently coating the seam with a resin mixture of a glycoluril resin and a polyol resin.

U.S. application Ser. No. 12/413,832, U.S. Publication No. 20100248104, filed Mar. 30, 2009, entitled Polyaniline Dialkylsulfate Complexes Containing Intermediate Transfer Members, the disclosure of which is totally incorporated herein by reference, illustrates an intermediate transfer member comprised of a polyaniline dialkylsulfate complex.

U.S. application Ser. No. 12/413,852, U.S. Publication No. 20100248102, filed Mar. 30, 2009, entitled Crosslinked Resin Mixture Backing Layer Containing Photoconductor, the disclosure of which is totally incorporated herein by reference, illustrates a photoconductor comprising a substrate, an imaging layer thereon, and a backing layer located on a side of the substrate opposite the imaging layer wherein the outermost layer of the backing layer adjacent to the substrate is comprised of a mixture of glycoluril resin and a polyacetal resin mixture.

Illustrated in U.S. application Ser. No. 12/200,147, U.S. Publication No. 20100055328, entitled Coated Seamed Transfer Member, filed Aug. 28, 2008, is a process which comprises providing a flexible belt having a welded seam extending from one parallel edge to the other parallel edge, the welded seam having a rough seam region comprising an overlap of two opposite edges; contacting the rough seam region with a heat and pressure applying tool; and smoothing out the rough seam region with heat and pressure applied by the heat and pressure applying tool to produce a flexible belt having a smooth welded seam, and subsequently coating the seam with a crosslinked acrylic resin.

Illustrated in U.S. application Ser. No. 12/200,179, U.S. Publication No. 20100051171, entitled Coated Transfer Member, filed Aug. 28, 2008, is a process which comprises providing a flexible belt having a welded seam extending from one parallel edge to the other parallel edge, the welded seam having a rough seam region comprising an overlap of two opposite edges; contacting the rough seam region with a heat and pressure applying tool; and smoothing out the rough seam region with heat and pressure applied by the heat and pressure applying tool to produce a flexible belt having a smooth welded seam, and subsequently coating the belt with a crosslinked acrylic resin.

Illustrated in U.S. application Ser. No. 11/895,255, U.S. Publication No. 20090050255, filed Aug. 22, 2007, the disclosure of which is totally incorporated here by reference, is a process for the post treatment of an ultrasonically welded seamed flexible imaging member belt comprising providing a flexible belt having a welded seam extending from one parallel edge to the other parallel edge, the welded seam having a rough seam region comprising an overlap of two opposite edges; positioning the flexible belt on a lower anvil such that the flexible belt is held in position on the lower anvil by vacuum; contacting the rough seam region with a heat and pressure applying tool; and smoothing out the rough seam region with heat and pressure applied by the heat and pressure applying tool to produce a flexible belt having a smooth welded seam without removing the seam material.

**BACKGROUND**

Disclosed are intermediate transfer members, and more specifically, coated intermediate transfer members useful in transferring a developed image in an electrostatographic, for example xerographic, including digital, image on image, and the like, printers, machines or apparatuses. In embodiments, there are selected, for example, a dual layered transfer member, such as a two layered intermediate transfer member comprised of a supporting substrate like a polyimide, and there-

after, applying onto the entire substrate surface a crosslinked mixture of a glycoluril resin and a polyol resin.

Intermediate transfer belts can be generated in the form of seamed belts fabricated by fastening two ends of a web material together, such as by welding, sewing, wiring, stapling, or gluing. While seamless intermediate transfer belts are known, they may require manufacturing processes that render them more costly as compared to similar seamed intermediate transfer belts.

Seamed belts can be fabricated from a sheet cut that originates from an imaging member web. The sheets are generally rectangular or in the shape of a parallelogram where the seam does not form a right angle to the parallel sides of the sheet. All edges may be of the same length or one pair of parallel edges may be longer than the other pair of parallel edges. The sheets are formed into a belt by joining overlapping opposite marginal end regions of the sheet. A seam is typically produced in the overlapping marginal end regions at the point of joining. Joining of the aforementioned areas may be effected by any suitable means, such as by welding, like ultrasonic welding, gluing, taping, pressure heat fusing, and the like.

Ultrasonic welding can be accomplished by retaining in a down position the overlapped ends of a flexible imaging member sheet with a vacuum against a flat anvil surface, and guiding the flat end of an ultrasonic vibrating horn transversely across the width of the sheet, over and along the length of the overlapped ends, to form a welded seam. Ultrasonically welding results in an overlap seam that has an irregular surface topology rendering it difficult for a cleaner blade to remove toner around the seam, and such welding can also cause damage to the cleaner blades by nicking the cleaning edge of the blade. In addition, toner trapping resulting from the poor cleaning and the blade damage causes streaking from the seam, and creates an image quality problem. Many post fabrication seam smoothing techniques, which remove material from the seam, may also degrade seam strength.

Also, when ultrasonically welded into a belt, the seam of a multilayered electrophotographic flexible imaging member belt may occasionally contain undesirable high protrusions such as peaks, ridges, spikes, and mounds. These seam protrusions present problems during image cycling of the belt because they interact with the cleaning blade causing blade wear and tear, which can affect cleaning blade efficiency and reduce service life.

In a typical electrostatographic reproducing apparatus, a light image of an original to be copied is recorded in the form of an electrostatic latent image upon a photosensitive member or photoconductor, and the latent image is subsequently rendered visible by the application of electroscopic thermoplastic resin particles and colorant. Generally, the electrostatic latent image is developed by a developer mixture comprised of carrier granules having toner particles adhering triboelectrically thereto, or a liquid developer material, which may include a liquid carrier having toner particles dispersed therein. The developer material is advanced into contact with the electrostatic latent image, and the toner particles are deposited thereon in image configuration. Subsequently, the developed image is transferred to a copy sheet. It is advantageous to transfer the developed image to a coated intermediate transfer web, belt or component, and subsequently transfer with very high transfer efficiency the developed image from the intermediate transfer member to a permanent substrate. The toner image is subsequently usually fixed or fused upon a support, which may be the photoconductor or other support such as plain paper.

In electrostatographic printing machines wherein the toner image is electrostatically transferred by a potential difference

between the imaging member and the intermediate transfer member, the transfer of the toner particles to the intermediate transfer member, and the retention thereof should be substantially complete so that the image ultimately transferred to the image receiving substrate will have a high resolution. Substantially about 100 percent toner transfer occurs when most or all of the toner particles comprising the image are transferred, and little residual toner remains on the surface from which the image was transferred.

Intermediate transfer members allow for a number of advantages such as enabling high throughput at modest process speeds, improving registration of the final color toner image in color systems using synchronous development of one or more component colors using one or more transfer stations, and increasing the variety of final substrates that can be used.

More specifically, a bump, surface irregularity, or other discontinuity in the seam of the belt may disturb the tuck of the cleaning blade as it makes intimate contact with the photoconductive member surface to effect residual toner and debris removal. The increased height differential may allow toner to pass under the cleaning blade, and not be cleaned. Furthermore, seams having differential heights may, when subjected to repeated striking by cleaning blades, cause photoconductive member cycling speed disturbance which adversely affects the crucial photoconductive belt motion quality. Moreover, seams with a bump or any morphological defects can cause the untransferred residual toner to be trapped in the sites of the seam surface irregularities. The seam of a photoreceptor belt, which is repeatedly subjected to the striking action by a cleaning blade under machine functioning conditions, can trigger the development of premature seam delamination failure. In addition, the discontinuity in belt thickness due to the presence of an excessive seam height yields variances of mechanical strength in the belt, and reduces the fatigue flex life of the seam when cycling over belt module support rollers. As a result, both the cleaning life of the blade, and the overall service life of the photoreceptor belt can be diminished.

Moreover, the protrusion high spots in the seam may also interfere with the operation of subsystems of copiers, printers, and duplicators by damaging electrode wires used in development that position the wires parallel to and closely spaced from the outer imaging surface of belt photoreceptors. These closely spaced wires are employed to facilitate the formation of a toner powder cloud at a development zone adjacent to a toner donor roll and the imaging surface of the belt imaging member.

In operation, an intermediate transfer belt is contacted with a toner image bearing member such as a photoreceptor belt. In the contact zone, an electrostatic field generating device, such as a corotron, a bias transfer roller, a bias blade, or the like, creates electrostatic fields that transfer toner onto the intermediate transfer belt. Subsequently, the intermediate transfer belt is brought into contact with a receiver. An electrostatic field generating device then transfers toner from the intermediate transfer belt to the receiver. Depending on the system, a receiver can be another intermediate transfer member or a substrate onto which the toner will eventually be fixed.

Regarding high speed printers, there is a need for a multi-layered member with separate functions for each layer. Typical multi-layered members comprises two layers, a polyimide bottom layer for reliable mechanical strength, and a functional top layer for high fidelity transfer, where the polyimide bottom layer can be either seamless or seamed.

More specifically, there is a need for a seamed dual layered member, such as a belt, that avoids or eliminates a number of

the disadvantages mentioned herein, and more specifically, there is a need for an ITB with excellent surface topology such that it can withstand dynamic fatigue conditions, and a need for further improving the transfer of an image, such as a xerographic image from a member like an intermediate transfer member to a substrate like paper, and where there is added to the top overcoat layer a component that possesses slippery characteristics such as a siloxane component or a fluoro component selected in an amount of from about 0.1 to about 5 weight percent. For example, the coated member as disclosed herein provides a smoother surface with substantially decreased or eliminated profile protrusions or irregularities thereby extending its service life. There is also a need for a substantially completely imageable seam, which avoids or minimizes the disadvantages indicated herein by overcoating the entire member inclusive of the seam or seams with a conductive polymer mixture layer, and which layer is mechanically robust and electrically matches the surface resistivity of the seamed intermediate transfer belt (ITB), or intermediate transfer member, which resistivity is from about  $10^9$  to about  $10^{13}$  ohm/sq.

## REFERENCES

Illustrated in U.S. Pat. No. 7,031,647 is an imageable seamed belt containing a lignin sulfonic acid doped polyaniline.

Illustrated in U.S. Pat. No. 7,139,519 is an intermediate transfer belt, comprising a belt substrate comprising primarily at least one polyimide polymer; and a welded seam.

Illustrated in U.S. Pat. No. 7,130,569 is a weldable intermediate transfer belt comprising a substrate comprising a homogeneous composition comprising a polyaniline in an amount of, for example, from about 2 to about 25 percent by weight of total solids, and a thermoplastic polyimide present in an amount of from about 75 to about 98 percent by weight of total solids, wherein the polyaniline has a particle size of, for example, from about 0.5 to about 5 microns.

Puzzle cut seam members are disclosed in U.S. Pat. Nos. 5,487,707; 6,318,223, and 6,440,515.

Illustrated in U.S. Pat. No. 6,602,156 is a polyaniline filled polyimide puzzle cut seamed belt, however, the manufacture of a puzzle cut seamed belt is labor intensive and very costly, and the puzzle cut seam, in embodiments, is sometimes weak. The manufacturing process for a puzzle cut seamed belt usually involves a lengthy in time high temperature and high humidity conditioning step. For the conditioning step, each individual belt is rough cut, rolled up, and placed in a conditioning chamber that is environmentally controlled at about 45° C. and about 85 percent relative humidity, for approximately 20 hours. To prevent or minimize condensation and watermarks, the puzzle cut seamed transfer belt resulting is permitted to remain in the conditioning chamber for a suitable period of time, such as 3 hours. The conditioning of the transfer belt renders it difficult to automate the manufacturing thereof, and the absence of such conditioning may adversely impact the belts electrical properties, which in turn results in poor image quality.

## SUMMARY

According to embodiments illustrated herein, there is provided a flexible intermediate member, such as a belt (ITB), that has an improved surface topology while maintaining the strength of the member, and processes for the preparation of flexible dual layered belts.

In embodiments, there is disclosed a process for the treatment, especially post treatment of an ultrasonically welded seamed flexible imaging member belt by overcoating a mixture layer where the seamed belt having at least one, such as 5 one, or two welded seams extending from one parallel edge to the other parallel edge, the welded seams having a rough seam region comprising an overlap of two opposite edges; positioning the flexible belt on a lower anvil such that the flexible belt is held in position on the lower anvil by a vacuum; 10 contacting the rough seam region with a heat and pressure applying tool; and smoothing out the rough seam region with heat and pressure being applied by the heat and pressure applying tool to produce a flexible belt having a smooth welded seam without removing seam material; and then subsequently 15 coating the entire flexible member with a mixture of resins as illustrated herein; and an intermediate transfer member, such as an intermediate transfer belt, comprised of a supporting substrate, and in contact with the substrate a resin mixture layer.

20 Embodiments illustrated herein also provide a process for the post treatment of an ultrasonically welded seamed flexible imaging member belt comprising providing a flexible belt having a welded seam extending from one parallel edge to the other parallel edge, the welded seam having a rough seam 25 region comprising an overlap of two opposite edges; positioning the flexible belt on a lower anvil such that the flexible belt is held in position on the lower anvil by a vacuum; contacting the rough seam region with a heat and pressure applying tool, the heat and pressure applying tool being selected from the group consisting of an ultrasonic vibrating horn, an automated heated pressure roller and a heated upper anvil; smoothing out the rough seam region with heat and 30 pressure to produce a flexible belt having a smooth welded seam; and thereafter overcoating the seam with the resin mixture illustrated herein; and a process which comprises providing a flexible belt having a welded seam extending from one parallel edge to the other parallel edge, the welded seam having a rough seam region comprising an overlap of two opposite edges; positioning the flexible belt on a lower anvil such that the flexible belt is held in position on the lower anvil by a vacuum; 35 contacting the rough seam region with a heat and pressure applying tool; and smoothing out the rough seam region with heat and pressure applied by the heat and pressure applying tool to produce a flexible belt having a smooth welded seam, and subsequently coating the entire member with the resin mixture illustrated herein.

## DETAILED DESCRIPTION

50 Aspects of the present disclosure relate to an intermediate transfer member comprised of a supporting substrate, and wherein the substrate is coated with a mixture of a glycoluril resin and a polyol resin; an intermediate transfer belt comprised of a supporting substrate, and in contact with the substrate a layer comprised of a mixture of a glycoluril resin and a polyol resin; a process which comprises providing a flexible belt having at least one welded seam extending from one parallel edge to the other parallel edge, the welded seam having a rough seam region comprising an overlap of two 55 opposite edges; contacting the rough seam region with a heat and pressure applying tool; and smoothing out the rough seam region with heat and pressure applied by the heat and pressure applying tool to produce a flexible belt having a smooth welded seam or seams, and subsequently coating the entire belt with a mixture of a glycoluril resin and a polyol resin; an intermediate transfer member comprised of a seamed substrate, and wherein the substrate is coated with a 60

65

mixture of a known glycoluril polymer and a known polyol polymer; a process which comprises providing a flexible belt having a welded seam extending from one parallel edge to the other parallel edge, the welded seam having a rough seam region comprising an overlap of two opposite edges; contacting the rough seam region with a heat and pressure applying tool; and smoothing out the rough seam region with heat and pressure applied by the heat and pressure applying tool to produce a flexible belt having a smooth welded seam, and subsequently coating the substrate inclusive of the seam or seams with a mixture of a commercially available glycoluril resin and a commercially available polyol resin; and an intermediate transfer member comprised of a double seamed substrate, and wherein the substrate inclusive of the seams are coated with a mixture of a glycoluril resin and a polyol resin, wherein the glycoluril resin is represented by the formula/structure illustrated herein, and the polyol resin is an acrylic polyol polymer generated by the polymerization of acrylic, derivatives of acrylic, methacrylic acid, derivatives of methacrylic acid, and other optional monomers, and mixtures thereof; an intermediate transfer member comprised of a supporting substrate and coated thereover a mixture of a glycoluril resin and a polyol resin; an intermediate transfer belt comprised of a double seamed substrate, and wherein the substrate is coated on from 95 to 100 percent of its surface area with a mixture of a glycoluril resin and a polyol resin; and a polymeric mixture coated member inclusive of flexible belts, fuser belts, pressure belts, intermediate transfer belts, transfuse belts, transport belts, developer belts, photoreceptor belts, and the like where the polymeric coating is comprised of a glycoluril resin and a polyol resin; and a belt with double welded seam, and where the entire belt is coated with a polymeric layer comprised of a glycoluril resin and a polyol resin.

Examples of the glycoluril resins are represented by the following formulas/structures



wherein each R substituent independently represents at least one of a hydrogen atom and an alkyl with, for example, 1 to about 18, from 1 to about 10, or from 1 to about 4 carbon atoms.

Examples of the glycoluril resin include unalkylated and highly alkylated glycoluril resin like CYMEL® and POWDERLINK® glycoluril resins commercially available from CYTEC Industries, Inc. Specific examples of the disclosed glycoluril resin include CYMEL® 1170 (a highly butylated resin with at least 75 percent of the R groups being butyl and the remainder of the R groups being hydrogen; viscosity=3,000 to 6,000 centipoise at 23° C.); CYMEL® 1171 (a highly methylated-ethylated with at least 75 percent of the R groups being methyl/ethyl and the remainder of the R groups being hydrogen, viscosity=3,800 to 7,500 centipoise at 23° C.); CYMEL® 1172 (an unalkylated resin with the R groups

being hydrogen); and POWDERLINK® 1174 (a highly methylated resin with at least 75 percent of the R groups being methyl and the remainder of the R groups being hydrogen, solid at 23° C.).

- 5 The number average molecular weight of the glycoluril resin is, for example, from about 200 to about 1,000 or from about 250 to about 600. The weight average molecular weight of the glycoluril resin is, for example, from about 230 to about 3,000 or from about 280 to about 1,800.
- 10 Examples of the polyol resin include acrylic polyol resins. In embodiments, acrylic polyol resin or acrylics examples include copolymers of derivatives of acrylic and methacrylic acid including acrylic and methacrylic esters and compounds containing nitrile and amide groups, and other optional monomers. The acrylic esters can be selected from, for example, the group consisting of n-alkyl acrylates wherein alkyl contains in embodiments from 1 to about 25 carbon atoms, such as methyl, ethyl, propyl, butyl, pentyl, hexyl, heptyl, octyl, nonyl, decyl, dodecyl, tetradecyl, or hexadecyl acrylate; secondary and branched-chain alkyl acrylates such as isopropyl, isobutyl, sec-butyl, 2-ethylhexyl, or 2-ethylbutyl acrylate; olefinic acrylates such as allyl, 2-methylallyl, furfuryl, or 2-butene acrylate; aminoalkyl acrylates such as 2-(dimethylamino)ethyl, 2-(diethylamino)ethyl, 2-(dibutylamino)ethyl, or 3-(diethylamino)propyl acrylate; ether acrylates such as 2-methoxyethyl, 2-ethoxyethyl, tetrahydrofurfuryl, or 2-butoxyethyl acrylate; cycloalkyl acrylates such as cyclohexyl, 4-methylcyclohexyl, or 3,3,5-trimethylcyclohexyl acrylate; halogenated alkyl acrylates such as 2-bromoethyl, 2-chloroethyl, or 2,3-dibromopropyl acrylate; glycol acrylates and diacrylates such as ethylene glycol, propylene glycol, 1,3-propanediol, 1,4-butanediol, diethylene glycol, 1,5-pantanediol, triethylene glycol, dipropylene glycol, 2,5-hexanediol, 2,2-diethyl-1,3-propanediol, 2-ethyl-1,3-hexanediol, or 1,10-decanediol acrylate, and diacrylate. Examples of methacrylic esters can be selected from, for example, the group consisting of alkyl methacrylates such as methyl, ethyl, propyl, isopropyl, n-butyl, isobutyl, sec-butyl, t-butyl, n-hexyl, n-octyl, isoctyl, 2-ethylhexyl, n-decyl, or tetradecyl methacrylate; unsaturated alkyl methacrylates such as vinyl, allyl, oleyl, or 2-propynyl methacrylate; cycloalkyl methacrylates such as cyclohexyl, 1-methylcyclohexyl, 3-vinylcyclohexyl, 3,3,5-trimethylcyclohexyl, bornyl, isobornyl, or cyclopenta-2,4-dienyl methacrylate; aryl methacrylates such as phenyl, benzyl, or nonylphenyl methacrylate; hydroxyalkyl methacrylates such as 2-hydroxyethyl, 2-hydroxypropyl, 3-hydroxypropyl, or 3,4-dihydroxybutyl methacrylate; ether methacrylates such as methoxymethyl, ethoxymethyl, 2-ethoxyethoxymethyl, allyloxymethyl, benzylloxymethyl, cyclohexyloxymethyl, 1-ethoxyethyl, 2-ethoxyethyl, 2-butoxyethyl, 1-methyl-(2-vinyl)ethyl, methoxymethoxyethyl, methoxyethoxyethyl, vinyloxyethoxyethyl, 1-butoxypropyl, 1-ethoxybutyl, tetrahydrofurfuryl, or furfuryl methacrylate; oxiranyl methacrylates such as glycidyl, 2,3-epoxybutyl, 3,4-epoxybutyl, 2,3-epoxyhexyl, or 10,11-epoxyundecyl methacrylate; aminoalkyl methacrylates such as 2-dimethylaminoethyl, 2-diethylaminoethyl, 2-t-octylaminoethyl, N,N-dibutylaminoethyl, 3-diethylaminopropyl, 7-amino-3,4-dimethyloctyl, N-methylformamidoethyl, or 2-ureidoethyl methacrylate; glycol dimethacrylates such as methylene, ethylene glycol, 1,2-propanediol, 1,3-butanediol, 1,4-butanediol, 2,5-dimethyl-1,6-hexanediol, 1,10-decanediol, diethylene glycol, or triethylene glycol dimethacrylate; trimethacrylates such as trimethylolpropane trimethacrylate; carbonyl-containing methacrylates such as carboxymethyl, 2-carboxyethyl, acetyl, oxazolidinylethyl, N-(2-methacryloyloxyethyl)-2-pyr-

olidinone, N-methacryloyl-2-pyrrolidinone, N-(metharyloyloxy)formamide, N-methacryloylmorpholine, or tris(2-methacryloxyethyl)amine methacrylate; other nitrogen-containing methacrylates such as 2-methacryloyloxyethylmethyl cyanamide, methacryloyloxyethyl trimethylammonium chloride, N-(methacryloyloxy-ethyl)diisobutylketimine, cyanomethyl, or 2-cyanoethyl methacrylate; halogenated alkyl methacrylates such as chloromethyl, 1,3-dichloro-2-propyl, 4-bromophenyl, 2-bromoethyl, 2,3-dibromopropyl, or 2-iodoethyl methacrylate; sulfur-containing methacrylates such as methylthiol, butylthiol, ethylsulfonylethyl, ethylsulfinylethyl, thiocyanatomethyl, 4-thiocyanatobutyl, methylsulfinylmethyl, 2-dodecylthioethyl methacrylate, or bis(methacryloyloxyethyl) sulfide; phosphorous-boron-silicon-containing methacrylates such as 2-(ethylenephosphino)propyl, dimethylphosphinomethyl, dimethylphosphonoethyl, diethylphosphatoethyl, 2-(dimethylphosphato)propyl, 2-(dibutylphosphono)ethyl methacrylate, diethyl methacryloylphosphonate, dipropyl methacryloyl phosphate, diethyl methacryloyl phosphite, 2-methacryloyloxyethyl diethyl phosphite, 2,3-butylene methacryloyl-oxyethyl borate, or methylidiethoxymethacryloyloxyethoxysilane. Methacrylic amides and nitriles can be selected from the group consisting of at least one of N methylmethacrylamide, N-isopropylmethacrylamide, N-phenylmethacrylamide, N-(2-hydroxyethyl) methacrylamide, 1-methacryloylamido-2-methyl-2-propanol, 4 methacryloylamido-4-methyl-2-pentanol, N-(methoxymethyl)methacrylamide, N-(dimethylaminoethyl)methacrylamide, N-(3-dimethylaminopropyl)methacrylamide, N-acetylmethacrylamide, N-methacryloylmaleamic acid, methacryloylamido acetonitrile, N-(2-cyanoethyl) methacrylamide, 1-methacryloylurea, N-phenyl-N-phenylethylmethacrylamide, N-(3-dibutylaminopropyl)methacrylamide, N,N-diethylmethacrylamide, N-(2-cyanoethyl)-N-methylmethacrylamide, N,N-bis(2-diethylaminoethyl)methacrylamide, N-methyl-N-phenylmethacrylamide, N,N'-methylenebis(methacrylamide), or N-(diethylphosphono)methacrylamide. Further optional monomer examples are styrene, acrolein, acrylic anhydride, acrylonitrile, acryloyl chloride, methacrolein, methacrylonitrile, methacrylic anhydride, methacrylic acetic anhydride, methacryloyl chloride, methacryloyl bromide, itaconic acid, butadiene, vinyl chloride, vinylidene chloride, or vinyl acetate.

Further specific examples of acrylic polyol resins include PARALOID<sup>TM</sup> AT-410 (acrylic polyol, 73 percent in methyl amyl ketone, Tg=30° C., OH equivalent weight=880, acid number=25, M<sub>w</sub>=9,000), AT-400 (acrylic polyol, 75 percent in methyl amyl ketone, Tg=15° C., OH equivalent weight=650, acid number=25, M<sub>w</sub>=15,000), AT-746 (acrylic polyol, 50 percent in xylene, Tg=83° C., OH equivalent weight=1,700, acid number=15, M<sub>w</sub>=45,000), AE-1285 (acrylic polyol, 68.5 percent in xylene/butanol=70/30, Tg=23° C., OH equivalent weight=1,185, acid number=49, M<sub>w</sub>=6,500) and AT-63 (acrylic polyol, 75 percent in methyl amyl ketone, Tg=25° C., OH equivalent weight=1,300, acid number=30), all available from Rohm and Haas, Philadelphia, Pa.; JONCRYL<sup>®</sup> 500 (styrene acrylic polyol, 80 percent in methyl amyl ketone, Tg=-5° C., OH equivalent weight=400), 550 (styrene acrylic polyol, 62.5 percent in PM-acetate/toluene=65/35, OH equivalent weight=600), 551 (styrene acrylic polyol, 60 percent in xylene, OH equivalent weight=600), 580 (styrene acrylic polyol, Tg=50° C., OH equivalent weight=350, acid number=10, M<sub>w</sub>=15,000), 942 (styrene acrylic polyol, 73.5 percent in n-butyl acetate, OH equivalent weight=400), and 945 (styrene acrylic polyol, 78

percent in n-butyl acetate, OH equivalent weight=310), all available from Johnson Polymer, Sturtevant, Wis.; RU-1100-1k<sup>TM</sup> with a M<sub>w</sub> of 1,000 and 112 hydroxyl value, and RU 1550-k5<sup>TM</sup> with a M<sub>w</sub> of 5,000 and 22.5 hydroxyl value, both available from Procachem Corp.; G-CURE<sup>TM</sup> 108A70, available from Fitzchem Corp.; NEOL<sup>®</sup> polyol, available from BASF; TONE<sup>TM</sup> 0201 polyol with a M<sub>w</sub> of 530, a hydroxyl number of 117, and acid number of <0.25, available from Dow Chemical Company.

10 The number average molecular weight of the polyol resin is, for example, from about 400 to about 50,000 or from about 1,000 to about 10,000. The weight average molecular weight of the polyol resin is, for example, from about 500 to about 100,000 or from about 1,500 to about 20,000. The polyol resin is present in an amount of, for example, from about 1 to about 99, about 10 to about 80 weight percent, or from about 30 to about 50 weight percent of the total overcoated layer components. By the addition of a small amount of an acid catalyst, the mixture of the glycoluril resin and the polyol 15 resin crosslinks upon thermal curing at temperatures of, for example, from about 80° C. to about 200° C. for a suitable time period, such as for example, from about 1 to about 60 minutes, and more specifically, curing at about 160° C. for 5 minutes, resulting in a mechanically robust mixture of a glycoluril resin and a polyol resin layer with a surface resistivity of from about 10<sup>9</sup> to about 10<sup>13</sup> ohm/sq, and specifically about 10<sup>11</sup> ohm/sq. While the percentage of crosslinking can be difficult to determine, and not being desired to be limited by theory, the mixture of the glycoluril resin and the polyol 20 resin layer is crosslinked to a suitable value, such as for example, from about 30 to about 100 percent, or from about 30 to about 50 percent.

25 The thickness of the overcoating comprised of the mixture of a glycoluril resin and a polyol resin is, for example, from about 1 to about 50 microns, from about 3 to about 30 microns, or from about 5 to about 15 microns.

30 The circumference of the transfer member in a film or belt configuration of from 1 to 2, or more layers is, for example, from about 250 to about 2,500 millimeters, from about 1,500 to about 2,500 millimeters, or from about 2,000 to about 2,200 millimeters. The width of the film or belt is, for example, from about 100 to about 1,000 millimeters, from about 200 to about 500 millimeters, or from about 300 to about 400 millimeters. The thickness of the film or belt is, for 35 example, from about 25 to about 500 microns, or from about 50 to 150 microns.

40 Nonlimiting examples of catalysts selected for the crosslinking of the polymeric mixture of a glycoluril resin and a polyol resin include oxalic acid, maleic acid, carboxylic acid, ascorbic acid, malonic acid, succinic acid, tartaric acid, citric acid, p-toluenesulfonic acid, methanesulfonic acid, and the like, and mixtures thereof. A typical concentration of acid catalyst is from about 0.01 to about 5 weight percent, about 45 0.5 to about 4 weight percent, and about 1 to about 3 weight percent based on the weight of the a mixture of a glycoluril resin and a polyol resin.

50 A blocking agent can also be included in the overcoat layer, which agent can "tie up" or substantially block the acid catalyst effect to provide solution stability until the acid catalyst function is initiated. Thus, for example, the blocking agent can block the acid effect until the solution temperature is raised above a threshold temperature. For example, some blocking agents can be used to block the acid effect until the solution temperature is raised above about 100° C. At that 55 time, the blocking agent dissociates from the acid and vaporizes. The unassociated acid is then free to catalyze the polymerization. Examples of such suitable blocking agents

include, but are not limited to, pyridine and commercial acid solutions containing blocking agents, such as CYCAT® 4045, available from Cytec Industries Inc.

The disclosed top layer further comprises an optional siloxane component or a fluoro component present in an amount of, for example, from about 0.1 to about 20 weight percent or from about 0.5 to about 5 weight percent, which component can be co-crosslinked with the glycoluril resin and polyol resin mixture thus providing further slippery characteristics to the top overcoat layer.

Examples of the crosslinkable siloxane components include hydroxyl derivatives of silicone modified polyacrylates such as BYK-SILCLEAN® 3700; polyether modified acryl polydimethylsiloxanes such as BYK-SILCLEAN® 3710; and polyether modified hydroxyl polydimethylsiloxanes such as BYK-SILCLEAN® 3720. BYK-SILCLEAN® is a trademark of BYK.

Examples of the crosslinkable fluoro component include (1) hydroxyl derivatives of perfluoropolyoxyalkanes such as FLUOROLINK® D (M.W. of about 1,000 and a fluorine content of about 62 percent), FLUOROLINK® D 10-H (M.W. of about 700 and fluorine content of about 61 percent), and FLUOROLINK® D10 (M.W. of about 500 and fluorine content of about 60 percent) (functional group —CH<sub>2</sub>OH); FLUOROLINK® E (M.W. of about 1,000 and a fluorine content of about 58 percent), and FLUOROLINK® E10 (M.W. of about 500 and fluorine content of about 56 percent) (functional group —CH<sub>2</sub>(OCH<sub>2</sub>CH<sub>2</sub>)<sub>n</sub>OH); FLUOROLINK® T (M.W. of about 550 and fluorine content of about 58 percent), and FLUOROLINK® T10 (M.W. of about 330 and fluorine content of about 55 percent) (functional group —CH<sub>2</sub>OCH<sub>2</sub>CH(OH)CH<sub>2</sub>OH); (2) hydroxyl derivatives of perfluoroalkanes (R<sub>f</sub>CH<sub>2</sub>CH<sub>2</sub>OH, wherein R<sub>f</sub>=F(CF<sub>2</sub>CF<sub>2</sub>)<sub>n</sub>) wherein n represents the number of groups, such as about 1 to about 50, such as ZONYL® BA (M.W. of about 460 and fluorine content of about 71 percent), ZONYL® BA-L (M.W. of about 440 and fluorine content of about 70 percent), ZONYL® BA-LD (M.W. of about 420 and fluorine content of about 70 percent), and ZONYL® BA-N (M.W. of about 530 and fluorine content of about 71 percent); (3) carboxylic acid derivatives of fluoropolyethers such as FLUOROLINK® E C (M.W. of about 1,000 and fluorine content of about 61 percent); (4) carboxylic ester derivatives of fluoropolymers such as FLUOROLINK® L (M.W. of about 1,000 and fluorine content of about 60 percent), FLUOROLINK® L10 (M.W. of about 500 and fluorine content of about 58 percent); (5) carboxylic ester derivatives of perfluoroalkanes (R<sub>f</sub>CH<sub>2</sub>CH<sub>2</sub>O(C=O)R, wherein R<sub>f</sub>=F(CF<sub>2</sub>CF<sub>2</sub>)<sub>n</sub>, and n is as illustrated herein, and R is alkyl) such as ZONYL® TA-N (fluoroalkyl acrylate, R=CH<sub>2</sub>=CH—, M.W. of about 570 and fluorine content of about 64 percent), ZONYL® TM (fluoroalkyl methacrylate, R=CH<sub>2</sub>=C(CH<sub>3</sub>)—, M.W. of about 530 and fluorine content of about 60 percent), ZONYL® FTS (fluoroalkyl stearate, R=C<sub>17</sub>H<sub>35</sub>—, M.W. of about 700 and fluorine content of about 47 percent), ZONYL® TBC (fluoroalkyl citrate, M.W. of about 1,560 and fluorine content of about 63 percent); (6) sulfonic acid derivatives of perfluoroalkanes (R<sub>f</sub>CH<sub>2</sub>CH<sub>2</sub>SO<sub>3</sub>H, wherein R<sub>f</sub>=F(CF<sub>2</sub>CF<sub>2</sub>)<sub>n</sub>, and n is as illustrated herein, such as ZONYL® TBS (M.W. of about 530 and fluorine content of about 62 percent); (7) ethoxysilane derivatives of fluoropolymers such as FLUOROLINK® S10 (M.W. of about 1,750 to about 1,950); and (8) phosphate derivatives of fluoropolymers such as FLUOROLINK® F10 (M.W. of about 2,400 to about 3,100). The FLUOROLINK® additives are available from Ausimont USA, and the ZONYL® additives are available from E.I. DuPont.

Examples of additional optional components present in the disclosed top layer include a number of known conductive components, such as polyaniline, carbon black or metal oxide, present in an amount of from about 0.1 to about 60 weight percent, from about 1 to about 30 weight percent, or from about 3 to about 15 weight percent.

In embodiments, the top layer polyaniline component has a relatively small particle size of, for example, from about 0.5 to about 5 microns, from about 1.1 to about 2.3 microns, from about 1.2 to about 2 microns, from about 1.5 to about 1.9 microns, or about 1.7 microns. Specific examples of polyanilines selected for the seam overcoat are PANIPOL™ F, commercially available from Panipol Oy, Finland; and lignosulfonic acid grafted polyaniline.

Examples of the top layer carbon blacks selected include VULCAN® carbon blacks, REGAL® carbon blacks, and BLACK PEARLS® carbon blacks available from Cabot Corporation. Specific examples of conductive carbon blacks are BLACK PEARLS® 1000 (B.E.T. surface area=343 m<sup>2</sup>/g, DBP absorption=105 ml/g), BLACK PEARLS® 880 (B.E.T. surface area=240 m<sup>2</sup>/g, DBP absorption=106 ml/g), BLACK PEARLS® 800 (B.E.T. surface area=230 m<sup>2</sup>/g, DBP absorption=68 ml/g), BLACK PEARLS® L (B.E.T. surface area=138 m<sup>2</sup>/g, DBP absorption=61 ml/g), BLACK PEARLS® 570 (B.E.T. surface area=110 m<sup>2</sup>/g, DBP absorption=114 ml/g), BLACK PEARLS® 170 (B.E.T. surface area=35 m<sup>2</sup>/g, DBP absorption=122 ml/g), VULCAN® XC72 (B.E.T. surface area=254 m<sup>2</sup>/g, DBP absorption=176 ml/g), VULCAN® XC72R (fluffy form of VULCAN® XC72), VULCAN® XC605, VULCAN® XC305, REGAL® 660 (B.E.T. surface area=112 m<sup>2</sup>/g, DBP absorption=59 ml/g), REGAL® 400 (B.E.T. surface area=96 m<sup>2</sup>/g, DBP absorption=69 ml/g), and REGAL® 330 (B.E.T. surface area=94 m<sup>2</sup>/g, DBP absorption=71 ml/g). Dibutyl phthalate (DBP) absorption by the voids within carbon blacks are used to measure the structure of carbon black. The higher the structure, the more the voids, and the higher is the DBP absorption.

Examples of the top layer metal oxide include tin oxide, antimony doped tin oxide, indium oxide, indium tin oxide, zinc oxide, and titanium oxide.

Supporting substrate layer examples are comprised of a number of known polymers and conductive components.

Examples of polymeric binders that in embodiments may be included in the intermediate transfer member substrate are polyimides (thermosetting or thermoplastic), polycarbonate, polyester such as poly(ethylene terephthalate) (PET), poly(ethylene naphthalate) (PEN) and poly(butylene terephthalate) (PBT), polypolyvinylidene fluoride (PVDF), polyethylene-co-polytetrafluoroethylene, polyamidimide, polyphenylene sulfide, polyamide, polysulfone, polyetherimide, polyester copolymer, rapidly cured polyimide polymers such as VTEC™ PI 1388, 080-051, 851, 302, 203, 201 and PETI-5, all available from Richard Blaine International, Incorporated, Reading, Pa. The thermosetting polyimides are cured at suitable temperatures, and more specifically, from about 180° C. to about 260° C. over a short period of time, such as, for example, from about 10 to about 120, and from about 20 to about 60 minutes; possess, for example, a number average molecular weight of from about 5,000 to about 500,000, or from about 10,000 to about 100,000, and a weight average molecular weight of from about 50,000 to about 5,000,000, or from about 100,000 to about 1,000,000; thermosetting polyimide precursors that are cured at higher temperatures (above 300° C.) than the VTEC™ PI polyimide precursors, and which precursors include, for example, PYRE-M.L® RC-5019, RC-5057, RC-5069, RC-5097,

RC-5053 and RK-692, all commercially available from Industrial Summit Technology Corporation, Parlin, N.J.; RP-46 and RP-50, both commercially available from Unitech LLC, Hampton, Va.; DURIMIDE® 100 commercially available from FUJIFILM Electronic Materials U.S.A., Inc., North Kingstown, R.I.; and KAPTON® HN, VN and FN, commercially available from E.I. DuPont, Wilmington, Del.; in amounts of, for example, from about 70 to about 97, or from about 80 to about 95 weight percent of the intermediate transfer member substrate layer.

Examples of specific selected thermoplastic polyimides are KAPTON® KJ, commercially available from E.I. DuPont, Wilmington, Del., as represented by



wherein x is equal to 2; y is equal to 2; m and n are from about 10 to about 300; and IMIDEX®, commercially available from West Lake Plastic Company, as represented by

first end marginal region is integral with the top surface, 25 generally including at least one layer immediately below, at and/or near the second end marginal region.



wherein  $z$  is equal to 1, and  $q$  is from about 10 to about 300.

Examples of polycarbonate binders selected include poly(4,4'-isopropylidene-diphenylene)carbonate (also referred to as bisphenol-A-polycarbonate), poly(4,4'-cyclohexylidine diphenylene)carbonate (also referred to as bisphenol-Z-polycarbonate), poly(4,4'-isopropylidene-3,3'-dimethyl-diphenyl)carbonate (also referred to as bisphenol-C-polycarbonate), and the like. In embodiments, the intermediate transfer member binders are comprised of bisphenol-A-polycarbonate resins, commercially available as MAKROLON®, with a weight average molecular weight of from about 50,000 to about 500,000.

Examples of the substrate conductive components include polyaniline, carbon black, or metal oxide present in an amount of from about 0.1 to about 60 weight percent, from about 1 to about 30 weight percent, or from about 3 to about 15 weight percent.

In embodiments, the substrate polyaniline component has a relatively small particle size of, for example, from about 0.5 to about 5 microns, from about 1.1 to about 2.3 microns, from about 1.2 to about 2 microns, from about 1.5 to about 1.9 microns, or about 1.7 microns. Specific examples of polyanilines selected for the seam overcoat are PANIPOL™ F, commercially available from Panipol Oy, Finland; and lignosulfonic acid grafted polyaniline.

Examples of the substrate metal oxide include tin oxide, antimony doped tin oxide, indium oxide, indium tin oxide, zinc oxide, and titanium oxide.

The end marginal regions of the transfer member can be joined by any suitable means including gluing, taping, stapling, pressure, and heat fusing to form a continuous member such as a belt, sleeve, or cylinder. Both heat and pressure can be used to bond the end marginal regions into a seam in the overlap region. The flexible member is thus transformed from a sheet of an intermediate transfer material into a continuous intermediate transfer belt, and which belt is then overcoated with the resin mixture illustrated herein. The flexible member has a first exterior major surface or side, and a second exterior major surface or side on the opposite side. The seam joins the flexible member so that the bottom surface, generally including at least one layer immediately above, at and/or near the

- 5
- 10

40 A heat and pressure seam joining means includes ultrasonic welding to transform the sheet of an intermediate transfer material into an intermediate transfer belt. The belt can be fabricated by ultrasonic welding of the overlapped opposite end regions of a sheet. In the ultrasonic seam welding process, 45 ultrasonic energy applied to the overlap region is used to melt suitable layers.

Ultrasonic welding is selected, in embodiments, for joining the flexible intermediate transfer member because it is rapid, clean and solvent free, and of low cost, and it produces a thin and narrow seam. In addition, ultrasonic welding is selected since the mechanical high frequency pounding of the welding horn causes the generation of heat at the contiguous overlapping end marginal regions of the flexible imaging sheet loop to maximize melting of one or more layers therein to form a strong and precisely defined seam joint. For example, ultrasonic welding, and an apparatus for performing the same is disclosed in U.S. Pat. No. 4,532,166, the disclosure of which is totally incorporated herein by reference.

In a specific embodiment, the heat and pressure applying tool is an ultrasonic vibrating horn. In such an embodiment, the lower anvil selected may be a flat anvil. This tool smoothes out the rough seam region by proceeding with a second welding pass across the welded region such that the rough seam region is further compressed under high pressure and heat.

65 Since the post treatment smoothing process uses the welding horn to further compress the overlap, rather than removing the protruding material, seam strength is not substantially

15

degraded. Moreover, the welded seam may be double welded from the back side of the seam as well. In such embodiments, the second welding pass is accomplished with the seam inverted on the anvil so that the imaging side of the belt is facing down on the anvil. In this manner, the overlap on the image side of the belt can be substantially eliminated as it conforms to the smooth surface of the anvil.

The heat and pressure applying tool is, in embodiments, an automated heated pressure roller or a heated upper anvil. In these embodiments, the lower anvil is a round anvil, and an edge of the seam region is positioned on an apex of the lower anvil, and where a smooth seam with no protrusion results by traversing the automated heated pressure roller along the seam to reform the edge of the seam region. The heated pressure roller applies pressure on the welded seam against the lower anvil while heating the seam such that a smooth welded seam is produced with the belt held in place by a vacuum on the lower anvil while the heated pressure roller traverses the seam. To effectively heat roll the seam smooth, the roller to the seam is positioned so as to be located on the apex of the anvil to fully expose the area to be smoothed. The surface of the roller should be tangent to the anvil's apex. Using a round anvil allows heat and pressure to be concentrated along the edge of the overlap. In further embodiments, the heated pressure roller is used in an automated system where the heated roller is affixed to a linear actuator, which drives it tangent to the roller's apex along its length. Temperature may be controlled by means of a thermostat controller while pressure may be controlled by spring tension.

By applying the heated upper anvil to the edge of the seam region, and where the welded seam is sandwiched between the upper and lower anvils, the welded seam is thus compressed under high pressure. Both the upper and lower anvils may be heated so that during the compression, the seam material is also heated close to its glass transition temperature to further facilitate the reformation of the welded seam and to produce a smooth welded seam. The upper and lower anvils may be heated by heating components embedded in the upper and lower anvils, and which are controlled by a thermostatic controller. In this embodiment, the welded seam may be reduced in seam thickness by from about 25 percent to about 35 percent.

The following Examples are provided.

#### COMPARATIVE EXAMPLE 1

A seamed intermediate transfer belt was prepared as follows. A 3 mil intermediate transfer sheet comprised of a mixture of 91 weight percent of KAPTON® KJ (available from E.I. DuPont), and 9 weight percent of polyaniline (1.7 microns in diameter size) was cut to a size of 362 millimeters wide by 2210.8 millimeters long. The ends were overlapped by 250 microns and an ultrasonic horn was used to compress the above mixture against a steel welding platen, melting the mixture in the overlap region, and creating a seam. The seam was then reverse welded, resulting in a seam of about 100 microns thick.

#### EXAMPLE I

The Comparative Example 1 seamed ITB is overcoated on the entire belt by a known flow coating method. The top layer

16

coating solution was prepared by introducing into an amber glass bottle in a weight ratio of 66:33:1 CYMEL® 1170, a highly butylated glycoluril resin shown as below



with R<sub>1</sub>, R<sub>2</sub> and R<sub>3</sub> being butyl, and R<sub>4</sub> being hydrogen; viscosity=3,000 to 6,000 centipoise at 23° C., commercially available from CYTEC Industries, Inc; JONCRYL® 580, a styrene acrylic polyol resin, T<sub>g</sub>32 50° C., OH equivalent weight=350, acid number=10, M<sub>w</sub>=15,000, commercially available from Johnson Polymers; and p-toluenesulfonic acid (pTSA). The resulting mixture was then dissolved in DOW-ANOL™ to form a solution containing 15 percent by weight solids.

The disclosed top layer crosslinked upon thermal curing at 160° C. for 5 minutes, resulting in a 20 micron, mechanically robust polymeric layer comprised of CYMEL® 1170/JONCRYL® 580/pTSA=66/33/1 with a surface resistivity of about 2.84×10<sup>11</sup> ohm/sq, which matched that of the ITB substrate layer. The surface resistivity of the top layer was measured using a High Resistivity Meter (Hiresa-Up MCP-HT450 from Mitsubishi Chemical Corp., under 1,000 V, averaging four measurements at varying spots, 72° F./65 percent room humidity).

The dual-layered seamed ITB of Example I and the non-coated seamed ITB of Comparative Example 1 are print tested on a Xerox Corporation DC8000 printer. After 100 prints, full page image quality analysis of 50 percent of the halftone images is visually evaluated, especially around the seam areas.

The Example I dual-layered seamed ITB has the advantages indicated. The seams were formed, as illustrated herein, by a first ultrasonic welding, and then turned upside down and welded a second time. The seam of the Example I dual-layered seamed ITB is invisible for 100 xerographic prints, while for the Comparative Example 1 ITB noncoated seam, the seam was visible for each of the 100 xerographic prints. The glycoluril resin/acrylic polyol resin Example I fully coated ITB is mechanically robust, and the seam remains invisible for 400,000 prints in contrast to the Comparative Example 1 ITB where the seam is visible beginning with the first print, and remains visible for 400,000 prints.

#### EXAMPLE II

The above process of Example I was repeated except that the top layer coating solution was prepared by introducing

17

into an amber glass bottle in a weight ratio of 66:32:1:1 CYMEL® 1170, a highly butylated glycoluril resin shown as below



with R<sub>1</sub>, R<sub>2</sub> and R<sub>3</sub> being butyl, and R<sub>4</sub> being hydrogen; viscosity=3,000 to 6,000 centipoise at 23° C., commercially available from CYTEC Industries, Inc; JONCRYL® 580, a styrene acrylic polyol resin, T<sub>g</sub>=50° C., OH equivalent weight=350, acid number=10. M<sub>w</sub>=15,000, commercially available from Johnson Polymers; p-toluenesulfonic acid (pTSA); and BYK-SILCLEAN® 3700, a hydroxyl derivative of silicone modified polyacrylate (siloxane component), commercially available from BYK. The resulting mixture was then dissolved in DOWANOL™ to form a solution containing 15 percent by weight solids.

The disclosed top layer crosslinked upon thermal curing at 160° C. for 5 minutes, resulting in a 20 micron, mechanically robust polymeric layer comprised of CYMEL® 1170/JONCRYL® 580/pTSAISILCLEAN® 3700=66/32/1/1 with a surface resistivity of about  $2.50 \times 10^{11}$  ohm/sq, which matched that of the ITB substrate layer.

The coefficients of kinetic friction of the top layers of Examples I and II against a polished stainless steel surface were measured by a COF Tester (Model D5095D, Dynisco Polymer Test, Morgantown, Pa.) according to ASTM D1894-63, procedure A. The tester was facilitated with a 2.5×2.5", 200 gram weight with rubber on one side, a moving polished stainless steel sled, and a DFGS force gauge (250 grams maximum). The top layers were cut into 2.5"×3.5" pieces and taped onto the 200 gram weight on the rubber side with the surfaces to be tested facing the sled. The coefficient of kinetic friction is defined as the ratio of the kinetic friction force (F) between the surfaces in contact to the normal force: F/N, where F was measured by the gauge and N is the weight (200 grams). The measurements were conducted at a sled speed of 6"/minute and at ambient conditions. Three measurements were performed for each seam coated ITB and their averages, and standard deviations are reported in Table 1.

TABLE 1

| Friction Coefficient |      |
|----------------------|------|
| Example I            | 0.39 |
| Example II           | 0.25 |

Incorporation of a siloxane component into the top layer (Example II) rendered the top layer about 40 percent more slippery than the Example I top layer without any siloxane component. The more slippery top layer is believed to be further beneficial to toner transfer and cleaning, resulting in an imageable seam and high fidelity transfer.

18

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others. Unless specifically recited in a claim, steps or components of claims should not be implied or imported from the specification or any other claims as to any particular order, number, 5 position, size, shape, angle, color, or material.

What is claimed is:

1. An intermediate transfer member consisting of a supporting substrate, and wherein said substrate is coated with a mixture in the configuration of a layer consisting of a glycoluril resin, a polyol resin, an optional conductive component, an optional catalyst, an optional siloxane component, and an optional fluoro component, and further consisting of 10 an optional release layer.

2. An intermediate transfer member in accordance with claim 1 wherein said substrate is a polymer selected from the group consisting of a polyimide, a polycarbonate, a polyamidimide, a polyphenylene sulfide, a polyamide, a polysulfone, a polyetherimide, a polyester or polyester copolymer, a polyvinylidene fluoride, a polyethylene-co-polytetrafluoroethylene, and mixtures thereof, and wherein said substrate includes a conductive component.

3. An intermediate transfer member in accordance with claim 1 wherein said substrate is comprised of a polyaniline, a carbon black, or a metal oxide.

4. An intermediate transfer member in accordance with claim 1 wherein said mixture of a glycoluril resin and a polyol resin contains from about 1 to about 99 weight percent of said glycoluril resin, and from 99 to about 1 weight percent of said polyol resin, and wherein the total thereof is about 100 percent.

5. An intermediate transfer member in accordance with claim 1 wherein said mixture of a glycoluril resin and a polyol resin contains from about 50 to about 85 weight percent of said glycoluril resin, and from 50 to about 15 weight percent of said polyol resin, and wherein the total thereof is about 100 percent.

6. An intermediate transfer member in accordance with claim 1 wherein said glycoluril resin is represented by



wherein each R group is at least one of hydrogen and alkyl.

7. An intermediate transfer member in accordance with claim 6 wherein said glycoluril resin possesses a number

19

average molecular weight of from about 200 to about 1,000 and a weight average molecular weight of from about 230 to about 3,000, and each R group is alkyl with from about 1 to about 4 carbon atoms.

8. An intermediate transfer member in accordance with claim 6 wherein said glycoluril resin possesses a number average molecular weight of from about 250 to about 600, and a weight average molecular weight of from about 280 to about 1,800, and each R is n-butyl, isobutyl, methyl, or ethyl.

9. An intermediate transfer belt in accordance with claim 6 wherein each of said R groups is hydrogen.

10. An intermediate transfer member in accordance with claim 6 wherein each of said R groups are alkyl with from 1 to about 10 carbon atoms.

11. An intermediate transfer member in accordance with claim 1 wherein said polyol resin is an acrylic polyol polymer generated from the polymerization of acrylic, derivatives of acrylic, methacrylic acid, derivatives of methacrylic acid, and mixtures thereof.

12. An intermediate transfer member in accordance with claim 11 wherein said derivatives of acrylic and said derivatives of methacrylic acid are selected from the group consisting of n-alkyl acrylates, secondary and branched-chain alkyl acrylates, olefinic acrylates, aminoalkyl acrylates, ether acrylates, cycloalkyl acrylates, halogenated alkyl acrylates, glycol acrylates and diacrylates, alkyl methacrylates, unsaturated alkyl methacrylates, cycloalkyl methacrylates, aryl methacrylates, hydroxyalkyl methacrylates, ether methacrylates, oxiranyl methacrylates, aminoalkyl methacrylates, glycol dimethacrylates, trimethacrylates, carbonyl-containing methacrylates, other nitrogen-containing methacrylates, halogenated alkyl methacrylates, sulfur-containing methacrylates, phosphorous-boron-silicon-containing methacrylates, N-methylmethacrylamide, N-isopropylmethacrylamide, N-phenylmethacrylamide, N-(2-hydroxyethyl) methacrylamide, 1-methacryloylamido-2-methyl-2-propanol, 4-methacryloylamido-4-methyl-2-pentanol, N-(methoxymethyl)methacrylamide, N-(dimethylaminoethyl) methacrylamide, N-(3-dimethylaminopropyl)methacrylamide, N-acetylmethacrylamide, N-methacryloylmaleamic acid, methacryloyl amidoacetonitrile, N-(2-cyanoethyl) methacrylamide, 1-methacryloylurea, N-phenyl-N-phenylethylmethacrylamide, N-(3-dibutylaminopropyl)methacrylamide, N,N-diethylmethacrylamide, N-(2-cyanoethyl)-N-methylmethacrylamide, N,N-bis(2-diethylaminoethyl)methacrylamide, N-methyl-N-phenylmethacrylamide, N,N'-methylenebismethacrylamide, N,N'-ethylenebismethacrylamide, or N-(diethylphosphono)methacrylamide, and mixtures thereof, and said optional monomers are selected from a group consisting of styrene, acrolein, acrylic anhydride, acrylonitrile, acryloyl chloride, methacrolein, methacrylonitrile, methacrylic anhydride, methacrylic acetic anhydride, methacryloyl chloride, methacryloyl bromide, itaconic acid, butadiene, vinyl chloride, vinylidene chloride, or vinyl acetate, and mixtures thereof.

13. An intermediate transfer member in accordance with claim 1 wherein said catalyst is an acid catalyst selected in an amount of from about 0.1 to about 2 weight percent, and said siloxane component or said fluoro component is present in an amount of from about 0.1 to about 5 weight percent.

14. An intermediate transfer member in accordance with claim 13 wherein said acid catalyst is a toluenesulfonic acid; said siloxane component is a hydroxyl derivative of silicone modified polyacrylate, a polyether modified acryl polydimethylsiloxane, a polyether modified hydroxyl polydimethylsiloxane, or an alkoxy silane of at least one alkoxy group bonding to at least one silicon atom; and said alkoxy is meth-

20

oxy, ethoxy, n-propoxy, isopropoxy, n-butoxy, or isobutoxy; and said fluoro component is at least one of hydroxyl derivatives of perfluoropolyoxyalkanes; hydroxyl derivatives of perfluoroalkanes; carboxylic acid derivatives of fluoropolymers; carboxylic ester derivatives of fluoropolymers; carboxylic ester derivatives of perfluoroalkanes; sulfonic acid derivatives of perfluoroalkanes; silane derivatives of fluoropolymers; and phosphate derivatives of fluoropolymers.

15. An intermediate transfer member in accordance with claim 1 wherein said outer release layer is positioned on said mixture layer.

16. An intermediate transfer member in accordance with claim 15 wherein said release layer is a fluorinated ethylene propylene copolymer, a polytetrafluoroethylene, a polyfluoroalkoxy polytetrafluoroethylene, a fluorosilicone, a copolymer or terpolymer of vinylidenefluoride, hexafluoropropylene and tetrafluoroethylene.

17. An intermediate transfer member in accordance with claim 1 wherein said substrate is a polymer selected from the group consisting of a polyimide, a polycarbonate, a polyamidimide, a polyphenylene sulfide, a polyamide, a polysulfone, a polyetherimide, a polyester, a polyvinylidene fluoride, and a polyethylene-co-polytetrafluoroethylene, and wherein said conductive component is a polyaniline, a carbon black, or a metal oxide; wherein said glycoluril resin is represented by



wherein each R group is at least one of hydrogen and alkyl wherein alkyl contains from 1 to about 6 carbon atoms; wherein said polyol resin is an acrylic polyol polymer and mixtures thereof; wherein said mixture of a glycoluril resin and a polyol resin includes said acid catalyst, said siloxane component, or said fluoro component; wherein said acid catalyst is a toluenesulfonic acid; said siloxane component is a hydroxyl derivative of a silicone modified polyacrylate, a polyether modified acryl polydimethylsiloxane, a polyether modified hydroxyl polydimethylsiloxane, or an alkoxy silane with at least one alkoxy group bonded to at least one silicon atom, and said alkoxy is methoxy, ethoxy, n-propoxy, isopropoxy, n-butoxy, or isobutoxy; and said fluoro component is at least one of hydroxyl derivatives of perfluoropolyoxyalkanes; hydroxyl derivatives of perfluoroalkanes; carboxylic acid derivatives of fluoropolymers; carboxylic ester derivatives of fluoropolymers; carboxylic ester derivatives of perfluoroalkanes; sulfonic acid derivatives of perfluoroalkanes; silane derivatives of fluoropolymers; or phosphate derivatives of fluoropolymers.

18. An intermediate transfer belt consisting of a supporting substrate, and in contact with said substrate a layer of a mixture of a glycoluril resin and a polyol resin, and wherein said mixture consists of about 50 to about 85 weight percent of said glycoluril resin, and from about 50 to about 15 weight

**21**

percent of said polyol resin, and wherein the total thereof is about 100 percent, and an optional catalyst and an optional conductive component.

**19.** An intermediate transfer belt in accordance with claim **18** wherein said substrate contains at least one seam. 5

**20.** An intermediate transfer member in accordance with claim **18** wherein said glycoluril resin is a butylated glycoluril formaldehyde resin present in an amount of from about 50 to about 90 weight percent, and said polyol resin is a styrene acrylic resin present in an amount of from about 50 to about 10 weight percent, wherein the total thereof is about 100 percent. 10

**21.** An intermediate transfer member in accordance with claim **18** wherein said substrate is a polymer selected from the group consisting of a polyimide, a polycarbonate, a polyamidimide, a polyphenylene sulfide, a polyamide, a polysulfone, a polyetherimide, a polyester, a polyvinylidene fluoride, a polyethylene-co-polytetrafluoroethylene, and mixtures 15 20

thereof, wherein said substrate includes said conductive component of a polyaniline, a carbon black, or a metal oxide; wherein said glycoluril resin is represented by



wherein each R group is at least one of hydrogen and alkyl wherein alkyl contains from 1 to about 4 carbon atoms; wherein said polyol resin is an acrylic polyol polymer.

\* \* \* \* \*